

## [54] METHOD FOR PRODUCING BITUMINOUS SUBSTANCE SUCH AS A COAL TARPATCH

[75] Inventors: Chiyozo Kishi; Mitsuo Tatsuta; Masayoshi Nago; Kanji Kibuishi; Yoshio Hatakeyama; Kaoru Miyakawa, all of Muroran, Japan

[73] Assignee: Nippon Steel Corporation, Tokyo, Japan

[22] Filed: Nov. 5, 1971

[21] Appl. No.: 196,096

## [30] Foreign Application Priority Data

Nov. 10, 1970 Japan..... 45/98979  
Nov. 10, 1970 Japan..... 45/98980  
Nov. 21, 1970 Japan..... 45/102970

[52] U.S. Cl..... 208/45, 208/6, 208/8, 208/39, 208/44

[51] Int. Cl..... C10c 3/02

[58] Field of Search ..... 208/8, 39, 44, 45, 208/6

## [56]

## References Cited

## UNITED STATES PATENTS

|           |         |                     |        |
|-----------|---------|---------------------|--------|
| 2,560,642 | 7/1951  | Greaves et al. .... | 208/44 |
| 3,490,586 | 1/1970  | Jaisle ....         | 208/45 |
| 1,722,872 | 7/1929  | Weindel....         | 208/45 |
| 2,299,469 | 10/1942 | D'Antal ....        | 208/44 |
| 3,692,663 | 9/1972  | Veda et al. ....    | 208/44 |

Primary Examiner—Delbert E. Gantz

Assistant Examiner—Veronica O'Keefe

Attorney—David Toren et al.

## [57]

## ABSTRACT

A method for producing bituminous substance such as coal tar pitch which comprises adding sulfuric acid to coal tar produced by a high temperature dry distillation of coal and a bituminous substance produced from the coal tar, then adding petroleum heavy oil to the mixture to precipitate and separate pitch component.

2 Claims, 2 Drawing Figures



PATENTED NOV 27 1973

3,775,289

SHEET 1 OF 2

FIG.1



INVENTORS

CHIYODO KISHI  
MITSUO TATSUTA  
MASAYOSHI NAGAO  
KANJI KIBUSHI  
KAORU MIYAKAWA  
YOSHIO HATAKEYAMA  
BY

*Foxon and McGeedy*  
ATTORNEYS

PATENTED NOV 27 1973

3,775,289

SHEET 2 OF 2

FIG.2



INVENTORS

CHIYOSHI KISHI  
MITSUO TATSUTA  
MASAYOSHI NAGAO  
KANJI KIBUCHI  
KAORU MIYAKAWA  
YOSHIO HATAKEYAMA

BY

*Toren and McGeady*  
ATTORNEYS

## METHOD FOR PRODUCING BITUMINOUS SUBSTANCE SUCH AS A COAL TAR PITCH

The present invention relates to improvements and relating to production of bituminous substance from coal tar such as pitch for pitch-coke and common pitches from coal tar.

According to a conventional method for producing bituminous substance such as pitch from coal tar, low boiling point aromatic components are removed by distillation or steaming, and if necessary poly-condensation reaction is caused by a heating treatment or by blowing in the air to a certain desired degree, or distilled oil from creosote oil and the like is cut back to obtain bituminous substance of desired properties (viscosity and softening point).

Further, although the air blowing-in or the addition of sulfur can promote the poly-condensation and increase benzole-insoluble component, these measures are nothing more than auxiliary means for the heating treatment since they are effective only under a heated condition between 300° to 400°C due to their reaction temperature.

Namely, it is impossible to blow in the air in an excessively large amount or to make addition of a large amount of sulfur in view of the softening temperature and so on.

Thus it has been eagerly sought for a method for improving the quality of pitches which can freely control the above properties, particularly the relation between the benzole-insoluble component and the quinoline-insoluble component.

The present inventors have completed a method for achieving the above object, in which waste sulfuric acid (waste sulfuric acid produced in the washing step with concentrated sulfuric acid of crude benzole and petroleum products and is called merely as waste sulfuric acid hereinafter) composed mainly of sulfonic acid and organic compounds of sulfuric acid, or concentrated sulfuric acid is used as catalyst for the polymerization improvement of pitches, and this method can achieve the object at a lower reaction temperature.

According to this method, it is possible to increase freely the benzole-insoluble component without increasing the quinoline-insoluble component, but this method has a defect that the increase in fixed carbon content which is an important factor showing the quality of pitches is rather small.

The present inventors have completed a method which overcomes completely the above defect by an extraction treatment using petroleum heavy oils.

It has been conventionally known that sludge-like product is precipitated when a petroleum solvent is added to pitches. But this precipitate contains a large amount of solvent and takes a form of rigid granular sludge, and thus can not be taken out as tar pitch continuously on a commercial scale. Accordingly it has never been contemplated to produce and utilize tar pitches by this method.

However, this method just mentioned has a problem in separation of the precipitating pitch component and the extracted petroleum solution, and under a certain condition a small amount of the petroleum heavy oil

mingles into the precipitating pitch component. In this case, the quality of pitch is shown by an excessive lowering of the fixed carbon content, and it is necessary to carefully establish the conditions such as the temperature, the mixing and extracting ratio, etc.

The present invention has also overcome this problem completely and makes it possible to produce pitches of good quality under a wide range of conditions in spite of differences in the quality of coal tar and properties of heavy oils.

In summary, the present invention is to provide a method which can maximize the extractability of low-molecular components and the separability of pitch component by using petroleum hydrocarbons containing or mixed with a small amount of low boiling point saturated hydrocarbon oil in addition to high boiling point petroleum heavy oil as extracting agent for removing low-molecular low-boiling point components in the coal tar.

20 The petroleum solvents used in the present invention have the following properties. The aniline point: more than 20°C (desirably more than 40°C). The boiling point range: the distillation ratio from the initial distillation point — 200°C is 0 — 30 percent, the distillation ratio from 200° — 360°C is 20 — 98 percent and the distillation ratio above 360°C is 0 — 80 percent.

25 The petroleum solvents within the above range include light oil, heavy oil, mixtures of light oil and heavy oil, mixtures of heavy oil with light oil, kerosene and gasoline, etc., and various crude oils.

30 When the extracting agent contains a low boiling point saturated hydrocarbon in addition to the high boiling point heavy oil, the separability is improved due to the lowering of viscosity at the time of extraction, 35 and part of paraffin or naphthene hydrocarbon oil which dissolves into the pitch layer in a very small amount is converted into a low boiling point hydrocarbon and thus distillation separation for final adjustment of softening point is easily attained.

40 When liquid petroleum gas or a low boiling point hydrocarbon oil (gasoline) alone is used as the extracting agent, it is necessary to give pressure in order to maintain the liquid phase, because of the heating which is required to take out the pitch component in the liquid form after the extraction, and extraction and separation of low molecular aromatic components which are unnecessary for the pitch is not satisfactory.

45 The present invention has eliminated the both defects and makes it possible to produce pitches of good quality from coal tar components with a simplified equipment.

50 The present invention shall be described in detail in reference to the attached drawings:

55 FIG. 1 is a graph showing the relation between the temperature and the viscosity of pitch produced by the present invention in comparison with that by a conventional method.

60 FIG. 2 is a graph showing the relation between the temperature and the viscosity of road tar produced by the present invention in comparison with that by a conventional method.

65 The references to heavy oils of grades A, B and C refer to the definitions of these grades pursuant to JIS (Japanese Industrial Standards) as follows:

| Category                          | Class 1(A)   |       | Class 2(B)   | Class 3(C) |       |           |               | Process for test (JIS) |
|-----------------------------------|--------------|-------|--------------|------------|-------|-----------|---------------|------------------------|
|                                   | No. 1        | No. 2 |              | No. 1      | No. 2 | No. 3     | No. 4         |                        |
| Reaction                          | Neutral      | →     | →            | Excess     | 70    | →         | →             | K2252.                 |
| Flash point, °C.                  | Excess 60    | →     | →            | 50-150     | →     | 150-400   | Less than 400 | K2265.                 |
| Kinematic viscosity (50° C.) est. | Less than 20 | →     | Less than 50 | 50-150     | →     | 150-400   | Less than 400 | K2282.                 |
| Pour point, °C.                   | Less than 5  | →     | Below 8      | Below 10   | →     | Below 1.5 | Below 2.0     | K2269.                 |
| Carbon residue, wt. percent       | Below 4      | →     | Below 8      | Below 0.5  | →     | Below 0.6 | Below 2.0     | K2270.                 |
| Moisture, vol. percent            | Below 0.3    | →     | Below 0.4    | Below 3.0  | →     | Below 3.5 | Below 1.5     | K2275.                 |
| S component, wt. percent          | Below 0.5    | →     | Below 2.0    | Below 0.5  | →     | Below 0.1 | →             | K2268 or 2273.         |
| Ash component, wt. percent        | Below 0.05   | →     | →            | →          | →     | →         | →             | K2272.                 |

## EXAMPLE 1

Petroleum heavy oil of C grade was added to coal tar in a ratio of 1 : 1 and the mixture was stirred at 50°C and 100°C respectively and left still at the above temperatures. The pitches thus separated have the following properties.

TABLE 1

| Treating temp., °C. | Softening point (Mercury method, °C.) | Percent      |                             |                         |
|---------------------|---------------------------------------|--------------|-----------------------------|-------------------------|
|                     |                                       | Fixed carbon | Benzole-insoluble component | Yield in respect to tar |
| 50                  | 44                                    | 39.6         | 10.5                        | 38                      |
| 100                 | 61                                    | 49.1         | 21.4                        | 32                      |

## EXAMPLE 2

The pitch produced by treating it at 50°C in Example 1 was further distilled, and thus obtained pitch has the following properties.

TABLE 2

| Distillation temp., °C. | Softening point (Mercury method, °C.) | Percent      |                             |                         |
|-------------------------|---------------------------------------|--------------|-----------------------------|-------------------------|
|                         |                                       | Fixed carbon | Benzole-insoluble component | Yield in respect to tar |
| Up to 340               | 67                                    | 50.6         | 23.2                        | 29                      |
| Up to 363               | 88                                    | 57.8         | 29.3                        | 25                      |

Analysis of properties of the material coal tar used in this example and the pitch produced by a conventional method are shown in Table 3.

TABLE 3

| Samples                                                             | Softening point (Mercury method, °C.) | Percent      |                             |                         |
|---------------------------------------------------------------------|---------------------------------------|--------------|-----------------------------|-------------------------|
|                                                                     |                                       | Fixed carbon | Benzole-insoluble component | Yield in respect to tar |
| Material coal tar                                                   | 30.4                                  | 4.5          | —                           | —                       |
| Pitches by conventional method:                                     | —                                     | —            | —                           | —                       |
| By mere distillation (1)...                                         | 67                                    | 46.5         | 12.1                        | 58                      |
| Same as (1) (2)...                                                  | 88                                    | 53.4         | 27.2                        | 66                      |
| Pitches by conventional method: Thermal poly-condensation treatment | 87                                    | 57.5         | 35.2                        | 57                      |

## EXAMPLE 3

The pitch produced by the treatment at 50°C in Example 1 was further treated at 150°C with addition of heavy oil of C grade in a ratio of 1 : 1. Pitch thus separated shows the following properties.

TABLE 4

| Softening point (Mercury method, °C.) | Percent      |                             |                         |
|---------------------------------------|--------------|-----------------------------|-------------------------|
|                                       | Fixed carbon | Benzole-insoluble component | Yield in respect to tar |
| 120                                   | 62.2         | 36.2                        | 11                      |

## EXAMPLE 4

Heavy oil of C grade was added to soft pitch and the mixture was stirred at 80°C and 150°C respectively. Pitches thus separated show the following properties.

TABLE 5

| Treating conditions              | Softening point, °C. | Percent      |                             |                               |
|----------------------------------|----------------------|--------------|-----------------------------|-------------------------------|
|                                  |                      | Fixed carbon | Benzole-insoluble component | Quinoline-insoluble component |
| Ratio of heavy oil to soft pitch | —                    | 34           | 38.8                        | 9.5                           |
| Material soft pitch              | —                    | 66           | 42.0                        | 27.4                          |
| 1/1                              | 80                   | 88           | 33.5                        | 8.2                           |
| 1/1                              | 150                  | 120          | 54.0                        | 9.5                           |
| 1/2                              | 150                  | 120          | 54.0                        | 9.0                           |

## EXAMPLE 5

Heavy oil of C grade was added to soft pitch in a ratio of 1 : 1 and the mixture was stirred at 150°C. Pitch thus separated was washed with gasoline and dried. The product shows the following properties.

TABLE 6

| Softening point, °C. | Percent      |                             |                               |
|----------------------|--------------|-----------------------------|-------------------------------|
|                      | Fixed carbon | Benzole-insoluble component | Quinoline-insoluble component |
| 71.0                 | 59.4         | 20.4                        | 0.4                           |

## EXAMPLE 6

Heavy oil of C grade was added to middle pitch in a ratio of 1 : 1 and the mixture was stirred and left still. Pitch thus separated has the following properties.

TABLE 7

| Samples                              | Softening point, °C. | Percent      |                             |                               |                           |
|--------------------------------------|----------------------|--------------|-----------------------------|-------------------------------|---------------------------|
|                                      |                      | Fixed carbon | Benzole-insoluble component | Quinoline-insoluble component | Specific gravity 38/38°C. |
| Middle pitch                         | 66.0                 | 46.5         | 12.1                        | 1.2                           | 1.263                     |
| Pitch treated with C grade heavy oil | 88.0                 | 54.5         | 32.7                        | 9.0                           | 1.285                     |

## EXAMPLE 7

A grade heavy oil, B grade heavy oil and C grade heavy oil were added to coal tar respectively in ratios shown in Table 8 and the mixtures were stirred and left still at 80°C. Soft pitch thus separated was distilled up to 320°C and thus obtained pitch has the following properties.

TABLE 8

| Tar/heavy oil ratio      | Softening point, °C. | Percent      |                             |                               |                              |
|--------------------------|----------------------|--------------|-----------------------------|-------------------------------|------------------------------|
|                          |                      | Fixed carbon | Benzole-insoluble component | Quinoline-insoluble component | Yield in respect to coal tar |
| A grade heavy oil, 1/0.5 | 91                   | 26.9         | 6.8                         | 50.6                          | 35                           |
| B grade heavy oil, 1/0.5 | 88                   | 25.2         | 5.1                         | 57.6                          | 30                           |
| C grade heavy oil, 1/1   | 92                   | 32.3         | 7.7                         | 58.7                          | 53                           |

## EXAMPLE 8

C grade heavy oil was added to coal tar in ratios of 1 : 1 and 1 : 0.5 and the mixtures were stirred and left still at 70°C and 50°C. Thus separated bituminous products were analyzed for their properties to meet the standards of road tars, and the results are shown under.

Table 10 shows the properties of the pitches produced by the present invention in comparison with those produced by the conventional method.

Further in FIG. 1, the curve 1 shows the temperature-

TABLE 12.—ADDITION OF WASTE SULFURIC ACID TO SOFT PITCH

| Addition of waste sulfuric acid, percent | Specific gravity, 30/30 C. | Softening point, °C. | Percent                     |                               |              |
|------------------------------------------|----------------------------|----------------------|-----------------------------|-------------------------------|--------------|
|                                          |                            |                      | Benzole-insoluble component | Quinoline-insoluble component | Fixed carbon |
| 0-----                                   | 1.229                      | 34.4                 | 9.53                        | 0.40                          | 38.38        |
| 1-----                                   | 1.243                      | 37.2                 | 17.56                       | 0.39                          | 40.43        |
| 2-----                                   | 1.249                      | 40.4                 | 21.66                       | 2.15                          | 42.56        |
| 3-----                                   | 1.278                      | 44.1                 | 25.13                       | 2.40                          | 42.60        |
| 5-----                                   | 1.291                      | 45.2                 | 34.37                       | 2.76                          | 42.73        |

TABLE 9

| Experiment No. | Tar/heavy oil ratio | Heavy oil treatment temperature, °C. | Yield of road tar, percent | Properties of road tars |                            |                  |                                 |                             |                  |
|----------------|---------------------|--------------------------------------|----------------------------|-------------------------|----------------------------|------------------|---------------------------------|-----------------------------|------------------|
|                |                     |                                      |                            | EVT, °C.                | Specific gravity, 25/25°C. | Acid oil content | Naphthalene-insoluble component | Toluene-insoluble component | Flash point, °C. |
| 1-----         | 1/1                 | 70                                   | 35                         | 60.4                    | 1.1182                     | 0.5              | 1.4                             | 16.3                        | 140 Good---      |
| 2-----         | 1/1                 | 50                                   | 40                         | 47.6                    | 1.165                      | 0.6              | 1.6                             | 11.8                        | 135 ---do---     |
| 3-----         | 1/0.5               | 70                                   | 37                         | 42.2                    | 1.162                      | 0.8              | 2.0                             | 10.2                        | 132 ---do---     |

TABLE 10

| Grade                              | Softening point (Hg method, °C.) | Percent                     |                               |              |
|------------------------------------|----------------------------------|-----------------------------|-------------------------------|--------------|
|                                    |                                  | Benzole-insoluble component | Quinoline-insoluble component | Fixed carbon |
| <b>Conventional method:</b>        |                                  |                             |                               |              |
| Middle pitch-----                  | 67                               | 12.1                        | 1.2                           | 46.5         |
| Hard pitch-----                    | 88                               | 27.2                        | 3.6                           | 53.4         |
| Hard pitch (modified by heat)----- | 87                               | 35.2                        | 10.0                          | 57.1         |
| <b>Inventive method:</b>           |                                  |                             |                               |              |
| Middle pitch (Example 2)-----      | 67                               | 23.2                        | 3.1                           | 50.6         |
| Middle pitch (Example 5)-----      | 71                               | 20.4                        | 0.4                           | 59.4         |
| Hard pitch (Example 2)-----        | 88                               | 29.3                        | 7.6                           | 57.8         |
| Hard pitch (Example 5)-----        | 91                               | 26.9                        | 6.8                           | 60.6         |

viscosity curve of a pitch produced by the conventional method (softening temperature 90°C, heat treatment) and the curve 2 shows the temperature-viscosity curve of a pitch produced by the present invention (softening temperature: 91.8°C, C grade heavy oil added in a ratio of 1 : 0.5, treated at 80°C).

As seen from FIG. 1, the pitch of the present invention shows lowered temperature-sensitivity as compared with that of the pitch produced by the conventional method. This tendency is also observed in road tar produced by the present invention, thus overcoming the defect of conventional road tar.

FIG. 2 shows measurements of the temperature-viscosity relation. 1 represents a viscosity-temperature curve of road tar produced by a conventional method (EUT 62°C) and 2 represents a viscosity-temperature curve of road tar produced by the present invention. As seen from FIG. 2 the temperature sensitivity of viscosity of road tar produced by the present invention is clearly lower than that by the conventional method.

## EXAMPLE 9

1 to 5 percent of waste sulfuric acid is added to middle pitch or soft pitch heated to 100° to 110°C, and stirring was given for 15 minutes. The results are shown in Tables 11 and 12.

TABLE 11.—ADDITION OF WASTE SULFURIC ACID TO MIDDLE PITCH

| Addition of waste sulfuric acid, percent | Specific gravity, 30/30 C. | Softening point, °C. | Percent                     |                               |              |
|------------------------------------------|----------------------------|----------------------|-----------------------------|-------------------------------|--------------|
|                                          |                            |                      | Benzole-insoluble component | Quinoline-insoluble component | Fixed carbon |
| 0-----                                   | 1.263                      | 66.0                 | 12.11                       | 1.22                          | 46.46        |
| 1-----                                   | 1.270                      | 72.2                 | 18.96                       | 2.46                          | 47.93        |
| 2-----                                   | 1.282                      | 75.0                 | 22.71                       | 2.86                          | 48.63        |
| 3-----                                   | 1.282                      | 77.7                 | 27.04                       | 2.99                          | 48.43        |
| 5-----                                   | 1.293                      | 78.7                 | 32.07                       | 2.40                          | 51.41        |

In this example, concentrated sulfuric acid and waste sulfuric acid are each added to coke oven tar and the mixtures are maintained at 50°, 80° and 120°C and stirred for 30 minutes.

TABLE 13.—ADDITION OF CONCENTRATED SULFURIC ACID TO TAR

| Amount of addition, percent | Analysis                                | Stirring temperature of— |        |         |
|-----------------------------|-----------------------------------------|--------------------------|--------|---------|
|                             |                                         | 50° C.                   | 80° C. | 120° C. |
| 0-----                      | Benzole-insoluble component, percent.   | 4.5                      | 4.5    | 4.5     |
| 0-----                      | Quinoline-insoluble component           | 1.8                      | 1.8    | 1.8     |
| 0-----                      | Fixed carbon percent                    | 30.4                     | 30.4   | 30.4    |
| 0-----                      | (Viscosity (60° C.) cp)                 | 200                      | 200    | 200     |
| 0.5-----                    | Benzole-insoluble component percent.    | 8.5                      | 8.2    | 9.1     |
| 0.5-----                    | Quinoline-insoluble component, percent. | 1.3                      | 1.9    | 1.4     |
| 0.5-----                    | Fixed carbon percent                    | 31.4                     | 32.5   | 32.3    |
| 0.5-----                    | (Viscosity (60° C.) cp)                 | 280                      | 360    | 580     |
| 1.0-----                    | Benzole-insoluble component, percent.   | 9.9                      | 12.2   | 13.6    |
| 1.0-----                    | Quinoline-insoluble component, percent. | 1.6                      | 1.2    | 1.5     |
| 1.0-----                    | Fixed carbon percent                    | 32.7                     | 32.8   | 34.0    |
| 1.0-----                    | (Viscosity (60° C.) cp)                 | 380                      | 740    | 1,060   |
| 3.0-----                    | Benzole-insoluble component, percent.   | 18.7                     | 23.5   | 25.2    |
| 3.0-----                    | Quinoline-insoluble component, percent. | 1.5                      | 1.5    | 1.2     |
| 3.0-----                    | Fixed carbon, percent                   | 33.4                     | 33.9   | 35.5    |
| 3.0-----                    | (Viscosity (60° C.) cp)                 | 720                      | 1,520  | —       |

TABLE 14.—ADDITION OF WASTE SULFURIC ACID TO TAR

| Amount of addition, percent | Analysis                                | Stirring temperature of— |        |         |
|-----------------------------|-----------------------------------------|--------------------------|--------|---------|
|                             |                                         | 50° C.                   | 80° C. | 120° C. |
| 0-----                      | Benzole-insoluble component, percent.   | 4.5                      | 4.5    | 4.5     |
| 0-----                      | Quinoline-insoluble component, percent. | 1.8                      | 1.8    | 1.8     |
| 0-----                      | Fixed carbon, percent                   | 30.4                     | 30.4   | 30.4    |
| 0-----                      | (Viscosity (60° C.) cp)                 | 200                      | 200    | 200     |
| 0-----                      | Benzole-insoluble component, percent.   | 8.9                      | 9.6    | 9.1     |
| 1.0-----                    | Quinoline-insoluble component, percent. | 1.4                      | 1.8    | 1.8     |
| 1.0-----                    | Fixed carbon, percent                   | 32.0                     | 33.1   | 34.6    |
| 1.0-----                    | (Viscosity (60° C.) cp)                 | 300                      | 420    | 930     |

Properties of waste sulfuric acid and concentrated sulfuric acid are shown Table 15.

TABLE 15

| Specific gravity, 15/4° C.      | Sulfuric acid concentration | Percent                                            |                                     |               |
|---------------------------------|-----------------------------|----------------------------------------------------|-------------------------------------|---------------|
|                                 |                             | Sulfonic acids and organic esters of sulfuric acid | Tar-like high polymerized substance | Water content |
| Waste sulfuric acid-----        | 1.48                        | 37                                                 | 31                                  | 28            |
| Concentrated sulfuric acid----- | 1.84                        | 95                                                 | —                                   | 5             |

Yields of pitch in case when waste sulfuric acid or concentrated sulfuric acid is added to tar are shown in Table 16.

| TABLE 16                               |                               |                                 | 5      |                      |      |
|----------------------------------------|-------------------------------|---------------------------------|--------|----------------------|------|
| Percent                                |                               | Percent                         |        |                      |      |
| Addition of concentrated sulfuric acid | Softening point of pitch, °C. | Addition of waste sulfuric acid | Yield  | Softening point, °C. |      |
| 0.....                                 | 60.4                          | 85.0                            | 0..... | 60.4                 | 85.0 |
| 1.....                                 | 66.6                          | 86.1                            | 1..... | 71.0                 | 85.4 |
| 3.....                                 | 82.9                          | 85.6                            | 3..... | 79.0                 | 85.1 |
| 5.....                                 | 88.7                          | 85.9                            | 5..... | 88.9                 | 85.7 |

TABLE 17.—PRODUCTION OF PITCH FROM TAR

| Experiment No. | Amount of added waste sulfuric acid, percent | Tar/heavy oil ratio | Grade of heavy oil | Heavy oil treatment temp., °C. | Yield of pitch, percent | Pitch properties     |                             |                               |         |
|----------------|----------------------------------------------|---------------------|--------------------|--------------------------------|-------------------------|----------------------|-----------------------------|-------------------------------|---------|
|                |                                              |                     |                    |                                |                         | Softening point, °C. | Benzole-insoluble component | Quinoline-insoluble component | Percent |
| 1.....         | 0                                            | 1/1                 | C                  | 80                             | 25                      | 88                   | 29.3                        | 9.2                           | 57.8    |
| 2.....         | 1.5                                          | 1/1                 | C                  | 80                             | 30                      | 95                   | 34.5                        | 9.5                           | 69.9    |
| 3.....         | 1.5                                          | 1/0.5               | C                  | 80                             | 28                      | 88                   | 36.5                        | 9.6                           | 69.6    |
| 4.....         | 1.5                                          | 1/0.5               | A                  | 80                             | 30                      | 91                   | 36.9                        | 9.4                           | 62.7    |
| 5.....         | 1.5                                          | 1/0.5               | B                  | 80                             | 28                      | 88                   | 35.2                        | 8.8                           | 58.6    |
| 6.....         | 5.0                                          | 1/1                 | C                  | 120                            | 46                      | 1 88                 | 1 58.2                      | 1 8.6                         | 1 51.0  |
| 7.....         | 5.0                                          | 1/1                 | C                  | 150                            | 36                      | 1 103                | 1 61.7                      | 1 8.9                         | 1 55.0  |
| 8.....         | 2.0                                          | 1/1                 | C                  | 50                             | 32                      | 111                  | 39.0                        | 8.7                           | 59.6    |
| 9.....         | 2.0                                          | 1/1                 | C                  | 80                             | 28                      | 87                   | 30.6                        | 9.5                           | 68.6    |
| 10.....        | 2.0                                          | 1/1                 | C                  | 80                             | 28                      | 89                   | 32.0                        | 9.4                           | 68.8    |

<sup>1</sup> Values for separated substances after heavy oil treatment without distillation for adjustment of softening point.

<sup>2</sup> Concentrated sulfuric acid.

TABLE 19.—RAW MATERIAL COAL TAR

| Specific gravity, 15/4°C. | Viscosity (60°C.) cp. | Percent      |                             |                               |                  | Fraction distillation test at— |
|---------------------------|-----------------------|--------------|-----------------------------|-------------------------------|------------------|--------------------------------|
|                           |                       | Fixed carbon | Benzole-insoluble component | Quinoline-insoluble component | Tar acid content |                                |
| 1.18.....                 | 200                   | 30.4         | 4.5                         | 0.4                           | 2.1              | 9.8 24 37                      |

EXAMPLE 11

In this example, waste sulfuric acid or concentrated sulfuric acid is added to tar produced from coke ovens, and after enough stirring, petroleum heavy oil is added to precipitate and separate pitch or aromatic bituminous substance of high molecule, and then distillation is effected to adjust the softening point.

This example is shown in Table 17 and Table 18.

TABLE 18.—PRODUCTION OF ROAD TAR FROM TAR

| Experiment No. | Amount of added waste sulfuric acid, percent | Tar/heavy oil ratio | Grade of heavy oil | Heavy oil treatment temp., °C. | Yield of road tar, percent | Properties of road tar |                            |                  |                                 | Fraction distillation test, percent at— |
|----------------|----------------------------------------------|---------------------|--------------------|--------------------------------|----------------------------|------------------------|----------------------------|------------------|---------------------------------|-----------------------------------------|
|                |                                              |                     |                    |                                |                            | EVT, °C.               | Specific gravity, 25/25°C. | Acid oil content | Naphthalene-insoluble component |                                         |
| 1.....         | 0                                            | 1/1                 | C                  | 70                             | 35                         | 60.4                   | 1.182                      | 0.5              | 2.8                             | 16.3 140 Good 0 4.7 9.1                 |
| 2.....         | 10                                           | 1/1                 | C                  | 70                             | 38                         | 63.2                   | 1.185                      | 0.4              | 2.7                             | 23.4 145 do 0 3.5 10.0                  |

REMARKS.—Separated substance (precipitate) after the heavy oil treatment was analysed as road tar and distillation or oil addition for adjustment of viscosity was not conducted.

TABLE 21.—PROPERTIES OF ROAD TAR BY CONVENTIONAL METHOD

| EVT, °C.  | Specific gravity, 15/4°C. | Properties of road tar |                                 |                  | Fraction distillation test at— |
|-----------|---------------------------|------------------------|---------------------------------|------------------|--------------------------------|
|           |                           | Acid oil content       | Naphthalene-insoluble component | Flash point, °C. |                                |
| 59.7..... | 1.23                      | 0.2                    | Trace...                        | 11.7             | 174 Good... 0 1.4 4.2          |

As seen from the Tables 17 and 18, the amount of added waste sulfuric acid or concentrated sulfuric acid has direct connection with increase and decrease of the benzole-insoluble component, and the proportion of heavy oil and the treatment temperature control the softening point, the fixed carbon content and separation from heavy oil.

The addition of heavy oil is preferably from 30 – 200 percent to the tar for good separation and accessibility

of precipitated pitch component, the temperature is preferably 50° to 150°C in case of tar and 100° to 250°C in case of middle pitch.

EXAMPLE 12

In this example concentrated sulfuric acid is added instead of waste sulfuric acid.

The raw material coal tar and, the properties of waste sulfuric acid and concentrated sulfuric acid, properties of pitch and road tar produced by this example are shown in Tables 19, 20, 21 and 22.

EXAMPLE 13

Extraction by petroleum light oil alone or mixed Oil

Petroleum light oil, heavy oil or mixed oil was added in various ratios to 10kg of coal tar, the mixtures were heated under stirring, left still and the pitch component which precipitated in the lower layer was analysed.

The results of this Example are shown in Table 22, and the material coal tar and the petroleum light oil and heavy oil used as solvent are set forth in Table 23.

TABLE 22

| Experiment No. | Extraction condition |                 |           | Properties of separated pitch |                      |              |                             |                               |                            |
|----------------|----------------------|-----------------|-----------|-------------------------------|----------------------|--------------|-----------------------------|-------------------------------|----------------------------|
|                | Mixing proportion    |                 |           | Temperature, °C.              | Softening temp., °C. | Percent      |                             |                               | Specific gravity, 30/30°C. |
|                | Coal tar             | C heavy oil (2) | Light oil |                               |                      | Fixed carbon | Benzole-insoluble component | Quinoline-insoluble component |                            |
| 1              | 1                    | 1               | 80        | 95.0                          | 63.1                 | 37.4         | 11.8                        | 1.34                          |                            |
| 2              | 1                    | 0.8             | 0.2       | 120                           | 98.7                 | 64.2         | 35.4                        | 11.0                          | 1.30                       |
| 3              | 1                    | 1               | 80        | 91.8                          | 58.7                 | 32.3         | 7.7                         | 1.28                          |                            |

TABLE 23

| Specific gravity, 15/4°C. | Initial boiling point, °C. | Fraction distillation test |         |         |         |           | Percent            |                             |                               |              |
|---------------------------|----------------------------|----------------------------|---------|---------|---------|-----------|--------------------|-----------------------------|-------------------------------|--------------|
|                           |                            | Percent at—                |         |         |         |           | Aniline point, °C. | Benzole-insoluble component | Quinoline-insoluble component | Fixed carbon |
|                           |                            | 200 °C.                    | 230 °C. | 300 °C. | 360 °C. | Dry point |                    |                             |                               |              |
| Coal tar                  | 1.200                      | 192                        | 15      | 21      | 34      |           |                    | 7.6                         | 3.4                           | 33.5         |
| Light oil                 | 0.811                      | 178                        | 12      | 65      | 87      |           | 34.2               | 68                          |                               |              |
| C heavy oil (2)           | 0.864                      | 238                        | 1       | 4       | 25      |           | 79                 |                             |                               |              |

It is also clear from the above results that a pitch having high fixed carbon content can be obtained when light oil together with C grade heavy oil is added than when C grade heavy oil above is added. Further the properties of the solvent and the extraction conditions have a great influence on the separability and properties of the pitch.

#### EXAMPLE 14

Properties of solvent in the solvent-extraction of coal tar and separability of pitch component.

Similar experiments as in Example 13 were conducted on various solvents, and the results are shown in Table 24.

TABLE 24

| Specific gravity, 15/4°C. | Aniline point, °C. | Fraction distillation test |             |         |         |           | Extraction condition |         |                                    | Fixed carbon in precipitated pitch, percent |  |
|---------------------------|--------------------|----------------------------|-------------|---------|---------|-----------|----------------------|---------|------------------------------------|---------------------------------------------|--|
|                           |                    | Initial boiling point, °C. | Percent at— |         |         | Dry point | Ratio                |         | Separability of precipitated pitch |                                             |  |
|                           |                    |                            | 200 °C.     | 300 °C. | 360 °C. |           | Coal tar             | Solvent | Temp., °C.                         |                                             |  |
| C heavy oil (1)           | 0.921              | 52                         | 232         | 21      |         |           | 1                    | 1       | 80                                 | Slightly poor..                             |  |
| Do                        | 0.921              | 52                         | 232         | 21      |         |           | 1                    | 0.5     | 80                                 | Poor..                                      |  |
| C heavy oil (2)           | 0.864              | 79                         | 238         | 25      |         |           | 1                    | 1       | 80                                 | Good..                                      |  |
| Do                        | 0.864              | 79                         | 238         | 25      |         |           | 1                    | 0.5     | 80                                 | Slightly poor..                             |  |
| B heavy oil               | 0.910              | 61                         | 180         | 13      | 56      |           | 1                    | 1       | 80                                 | Good..                                      |  |
| A heavy oil               | 0.839              | 72                         | 212         | 12      | 93      | 364       | 1                    | 1       | 80                                 | do..                                        |  |
| Light oil                 | 0.811              | 68                         | 178         | 12      |         | 342       | 1                    | 1       | 80                                 | do..                                        |  |
| Kerosene                  | 0.788              | 42                         | 170         | 46      |         | 233       | 1                    | 1       | 100                                | Slightly poor..                             |  |
| Gasoline                  | 0.736              | 10                         | 48          |         |         | 197       | 1                    | 1       | 30                                 | Poor..                                      |  |
| Crude oil                 | 0.853              | 54                         | 72          | 20      | 63      |           | 1                    | 1       | 80                                 | Good..                                      |  |
| Mixed oil (1)             | 0.826              | 77                         | 60          | 18      | 50      |           | 1                    | 1       | 80                                 | do..                                        |  |
| Mixed oil (2)             | 0.866              | 19                         | 64          | 30      | 64      |           | 1                    | 1       | 80                                 | Poor..                                      |  |

Remark: Aniline point was measured with distilled oil up to 360°C.

The mixed oil is a mixture of C grade oil, light oil, kerosene and gasoline.

As understood from the above results, it is a prerequisite for increasing the fixed carbon content in the separated pitch that the aniline point is high and a suitable amount of low-boiling point component is mixed.

According to the solvent-extraction of the present invention, the fixed carbon content in the pitch is increased, but the contents of benzole-insoluble component and B-resin component depend on the properties of the raw material coal tar because poly-condensation modification step by a heat treatment is not included as in the conventional method.

For solving the above problem, the present inventors have completed a method for producing pitch of very good quality by conducting poly-condensation after the addition of a small amount of waste sulfuric acid or concentrated sulfuric acid to coal tar at a low temperature. One example of this method is set forth under.

#### EXAMPLE 15

Extraction after the treatment with addition of waste sulfuric acid

10 kg of coal tar was heated between 50° and 80°C, 0.5 to 1.0 percent of waste sulfuric acid was added thereto, stirred fully, then crude oil or mixed oil was added in a ratio from 0.5 to 1.0 : 1 of the tar, maintained between 80° and 120°C, stirred and left still. The properties of thus separated pitch are shown in Table 25 (the adjustment of softening point was made by distillation).

TABLE 25

| Solvents  | Addition of waste sulfuric acid, percent | Solvent ratio |                        |     | Extraction temperature, °C. | Softening point, °C. | Fixed carbon | Benzole-insoluble component | Quinoline-insoluble component | Yield of pitch in respect to tar, percent |
|-----------|------------------------------------------|---------------|------------------------|-----|-----------------------------|----------------------|--------------|-----------------------------|-------------------------------|-------------------------------------------|
|           |                                          | Coal tar      | Crude oil or mixed oil |     |                             |                      |              |                             |                               |                                           |
|           |                                          |               |                        |     |                             |                      |              |                             |                               |                                           |
| Crude oil | 0.5                                      | 1             | 1                      | 80  | 90                          | 61.0                 | 33.8         | 11.0                        | 22.8                          | 34                                        |
| Do        | 0.5                                      | 1             | 1                      | 80  | 87                          | 59.6                 | 35.8         | 8.5                         | 27.3                          | 48                                        |
| Do        | 0.5                                      | 1             | 1                      | 120 | 93                          | 62.3                 | 42.0         | 11.5                        | 30.5                          | 30                                        |
| Do        | 0.5                                      | 1             | 0.5                    | 80  | 92                          | 61.0                 | 36.8         | 11.0                        | 25.8                          | 36                                        |
| Mixed oil | 0.5                                      | 1             | 0.5                    | 80  | 89                          | 58.1                 | 31.0         | 8.3                         | 22.7                          | 47                                        |
| Do        | 0.5                                      | 1             | 0.5                    | 80  | 88                          | 59.0                 | 37.5         | 8.1                         | 29.4                          | 51                                        |
| Do        | 1.0                                      | 1             | 0.5                    | 80  | 85                          | 56.5                 | 35.1         | 6.6                         | 28.5                          | 55                                        |
| Do        | 0.5                                      | 1             | 1                      | 80  | 96                          | 59.8                 | 36.1         | 8.2                         | 27.9                          | 49                                        |
| Do        | 0.5                                      | 1             | 0.5                    | 120 | 93                          | 62.0                 | 39.6         | 10.0                        | 29.6                          | 41                                        |

As above, the addition of waste sulfuric acid improves not only the benzole-insoluble component and  $\beta$  resin component, but also the yield of pitch.

These effects are same when sulfuric acid is used instead of waste sulfuric acid. Table 26 shows the analysis of the waste sulfuric acid used in this example.

from the coal tar B. But by mixing light oil etc. to the solvent and further by adding waste sulfuric acid thereto, it is possible to produce pitch of high grade.

It is also possible to apply the present inventive method to a soft pitch and a middle pitch as well as to the coal tar. This is shown in the following example.

TABLE 28

| Coal tar grade | Addition of waste sulfuric acid | Addition ratio to 1 of tar |           | Extraction temp., °C. | Properties of pitch  |              |                             |
|----------------|---------------------------------|----------------------------|-----------|-----------------------|----------------------|--------------|-----------------------------|
|                |                                 | C heavy oil                | Light oil |                       | Softening point, °C. | Fixed carbon | Benzole-insoluble component |
| B              | 1                               | -----                      | -----     | 80                    | 92                   | 58.7         | 32.3                        |
|                | 1                               | -----                      | -----     | 80                    | 97                   | 54.3         | 27.3                        |
|                | 0.5                             | 0.5                        | -----     | 80                    | 92                   | 58.5         | 32.1                        |
| A              | 1.0                             | 0.25                       | 0.25      | 80                    | 91                   | 56.5         | 34.1                        |
|                | 1.0                             | 0.25                       | 0.25      | 100                   | 97                   | 56.5         | 37.1                        |
|                | 1.0                             | -----                      | 0.5       | 80                    | 90                   | 59.1         | 41.1                        |

TABLE 26.—ANALYSIS OF WASTE SULFURIC ACID

| Specific gravity, 15/4 °C. | Percent               |                                              |       |       |
|----------------------------|-----------------------|----------------------------------------------|-------|-------|
|                            | Sulfuric acid content | Sulfonic acid, organic sulfonated substances | Tar   | Water |
| 1.485                      | 52.23                 | 28.07                                        | 14.29 | 54.1  |

25

## EXAMPLE 17

## Middle pitch and soft pitch

20 The experiment was conducted in the same manner as in the previous example except that 10 kg of a middle pitch or soft pitch was used instead of the coal tar, and C grade heavy oil alone or a mixed oil of light oil was used as extraction solvent. The results are shown in Table 29.

TABLE 29

| Bituminous material | Solvent ratio to 1 of material |           | Extraction temp., °C. | Properties of separated pitch |              |                             |
|---------------------|--------------------------------|-----------|-----------------------|-------------------------------|--------------|-----------------------------|
|                     | C heavy oil                    | Light oil |                       | Softening point, °C.          | Fixed carbon | Benzole-insoluble component |
| Middle pitch        | -----                          | -----     | 66.9                  | 46.5                          | 12.1         | 1.2                         |
| Do.                 | 1.0                            | -----     | 150                   | 88.0                          | 54.5         | 32.7                        |
| Do.                 | 0.8                            | 0.2       | 150                   | 89.1                          | 56.8         | 34.1                        |
| Soft pitch          | 1.0                            | -----     | 150                   | 78.1                          | 56.4         | 31.5                        |
| Do.                 | 0.8                            | 0.2       | 150                   | 80.0                          | 57.0         | 33.5                        |
|                     |                                |           |                       |                               |              | 0.4                         |

As seen from the above, when the poly-condensation treatment with addition of sulfuric acid and the solvent in the solvent-extraction are selected suitably it is possible to produce an electrode pitch of high grade from a

For comparison, the quality of the pitch produced by the present invention and the quality of the pitch produced by conventional methods are set forth in Table 30.

TABLE 30

| Producing method                                    | Properties of pitches |              |                             |                               |         |
|-----------------------------------------------------|-----------------------|--------------|-----------------------------|-------------------------------|---------|
|                                                     | Softening point, °C.  | Fixed carbon | Benzole-insoluble component | Quinoline insoluble component | Percent |
| Mere distillation by conventional method            | 67                    | 46.5         | 12.1                        | 1.5                           | 10.6    |
| Same as above but with modification by heating      | 87                    | 57.5         | 35.2                        | 10.7                          | 24.5    |
| Present invention, mixed oil used                   | 89                    | 58.1         | 31.0                        | 8.3                           | 22.7    |
| Present invention, waste sulfuric acid added (0.3%) | 88                    | 59.0         | 37.5                        | 8.1                           | 29.4    |
|                                                     |                       |              |                             |                               | Do.     |

raw material coal tar having low contents of fixed carbon and solvent-insoluble components.

The effects of the present invention due to difference in coal tar qualities are set forth in the next example.

## EXAMPLE 16

## Differences due to the qualities of material coal tars.

TABLE 27.—PROPERTIES OF MATERIAL COAL TAR

| Coal tar grade | Specific gravity, 15/4 °C. | Percent      |                             |                               |
|----------------|----------------------------|--------------|-----------------------------|-------------------------------|
|                |                            | Fixed carbon | Benzole-insoluble component | Quinoline insoluble component |
| A              | 1.157                      | 25.8         | 3.0                         | 0.5                           |
| B              | 1.200                      | 33.5         | 7.6                         | 3.4                           |

The experiment method is just same as in Example 15, and the results are shown in Table 28.

The results in Table 28 show that it is harder to produce pitch of good quality from the coal tar A than

From the above examples it is understood that according to the present invention it is possible to produce a high grade pitch containing high fixed carbon content and benzole-insoluble component content (namely high in  $\beta$ -resin component content) without requiring a high temperature treatment with a low-cost equipment, thus the present invention has very large economical advantage.

Further by using petroleum crude oil, as solvent, it is 60 possible to produce pitch at a very low cost, and the solvent after the extraction is a mixture of crude oil and low-molecular aromatic component of the coal tar, and thus can be readily used for production of petroleum products (gasoline, light oil, heavy oil and asphalt) by distillation.

Further, these petroleum products are enhanced in their qualities when mixed with aromatic component. For example, gasoline shows increase octane rating,

and asphalt shows improved mixability with aggregate materials and improved permeability when used for road pavement.

Also, the addition of waste sulfuric acid or sulfuric acid serves to prevent colouration of distilled oil and formation of gum substance at the time of distillation refinement of the separated extraction solvent and contributes for desulfurization, thus improving the quality of distilled products.

Although the object of the present invention is to provide a method for producing and improving coal tar, it is possible to produce unique petroleum products and low-sulfur fuel oil when coal tar is used as fuel or when the present invention is applied to the refining step of petroleum without heat decomposition and contact decomposition as conventionally done.

What is claimed:

1. A method for producing coal tar pitch comprising adding sulfuric acid to coal tar produced by the high temperature, dry distillation of coal and then adding a

20

petroleum hydrocarbon oil to the mixture, said oil having an aniline point above 20°C and consisting of 0-30 percent of a fraction having a boiling point up to 200°C, 20 to 98 percent of a fraction having a boiling point between 200° and 360°C and 0 to 80 percent of a fraction having a boiling point above 360°C, the ratio of coal tar to said oil being from 1:0.3 to 2.0, and maintaining the temperature between 50° and 250°C to precipitate and separate the pitch component.

10 2. A method for improving coal tar pitch by extraction comprising adding to the pitch a hydrocarbon oil having an aniline point above 20°C and consisting of 0-30 percent of a fraction having a boiling point up to 200°C, 20 to 98 percent of a fraction having a boiling point between 200° and 360°C and 0 to 80 percent of a fraction having a boiling point above 360°C, the ratio of coal tar to said oil being from 1:0.3 to 2.0, and maintaining the temperature between 50° and 250°C to precipitate and separate the pitch component.

\* \* \* \* \*

25

30

35

40

45

50

55

60

65